

C. ROBINSON.

PROCESS OF ORE TREATMENT.

APPLICATION FILED NOV. 29, 1910. RENEWED DEC. 1, 1913.

1,105,102.

Patented July 28, 1914.



Witnesses  
J. H. Gram  
S. Jay Teller



Fig. 1.



Inventor  
C. Robinson  
By  
D. A. Bliss  
Attorney

# UNITED STATES PATENT OFFICE.

CYRUS ROBINSON, OF MOUNT VERNON, NEW YORK, ASSIGNOR TO METALLURGICAL ENGINEERING & PROCESS CORPORATION, A CORPORATION OF NEW YORK.

## PROCESS OF ORE TREATMENT.

1,105,102.

Specification of Letters Patent. Patented July 28, 1914.

Application filed November 29, 1910, Serial No. 594,703. Renewed December 1, 1913. Serial No. 804,114.

*To all whom it may concern:*

Be it known that I, CYRUS ROBINSON, a subject of the King of Great Britain and Ireland, residing at Mount Vernon, in the county of Westchester and State of New York, have invented certain new and useful Improvements in Processes of Ore Treatment, of which the following is a specification, reference being had therein to the accompanying drawing.

This invention relates to improvements in processes of ore treatment and more especially to processes in which pulverized ore is first mixed with solvent solution to be acted upon, then separated from the solution and then subjected to the action of a second solvent solution.

One of the objects of my invention is to provide a process of this character in which the ore is mixed with a second solvent in an improved and novel manner.

Other objects will appear from the following specification.

In the accompanying drawings I have indicated more or less diagrammatically one form of apparatus which may be used in carrying out my improved process. This apparatus is similar in some respects to that disclosed in co-pending applications by myself and Robert S. Towne, for improvements in processes for extracting metals from ores, filed July 14, 1910, Serial No. 572,024, and for improvements in apparatus for extracting metals from ores, filed Jan. 24, 1911, Ser. No. 604,176. It will be understood, however, that this apparatus which is shown in the drawings has been selected merely by way of illustration and that other forms of apparatus may be equally well adapted for carrying out my present invention.

Of the drawings Figure 1 is a diagrammatic view of one form of apparatus which is adapted to be used in carrying out my invention. Fig. 2 is an enlarged fragmentary view showing a part of one of the dehydrators shown in Fig. 1.

In reading the following specification it can be considered as descriptive of a potassium cyanid process, but it will be apparent that the process described is equally

applicable to the extraction of ore values by other chemicals such as are well known in the art. Referring to the drawing, A indicates a tube mill or other preferred form 55 of reducing apparatus. To this mill the ore to be treated is supplied and at the same time there is supplied to the mill a solvent solution from a receptacle B. After the ore has been pulverized and intimately 60 mixed with the solution in the tube mill, it passes, together with the solution, to a receptacle indicated by C. This receptacle C may be of any desired type but it is preferably provided with means such as mechanical stirrers or jets of air or liquid such as additional solvent solution for agitating the mixture and insuring rapid action of the solvent on the ore. After the treatment in the receptacle C is complete the mixture of 70 ore and solvent solution passes to a dehydrator indicated by D. This dehydrator may be of any of a number of forms, but that which I now prefer and which I have diagrammatically indicated in the drawing 75 is shown and claimed in my co-pending application for dehydrators, filed Nov. 29, 1910, Serial No. 594,704. This dehydrator comprises a tank in which the mixture of ore and solution is contained, and a rotating 80 drum partly submerged in the mixture within the tank, the drum having its circumference made up of a filtering medium and being provided with means for connecting the inner surface of the medium with a vacuum 85 during certain parts of the revolution. A pump D' may be provided for maintaining the vacuum. As a result of this vacuum on the inner side of the filtering medium, the liquid constituent of the mixture in the 90 tank is drawn into the drum and out through a pipe such as D<sup>2</sup> connected with the vacuum pump. At one side of the drum there is provided a trough D<sup>3</sup>. A scraper or deflector D<sup>4</sup> engages the surface of the drum 95 and deflects material from it into the trough.

At D<sup>5</sup> there is provided one or more pipes extending longitudinally of the drum and having longitudinal rows of apertures directed toward the drum surface. The pipes at 100 D<sup>5</sup> are connected with a suitable source from which a fresh solvent solution under pres-

sure may be supplied. This fresh solution serves to break down and wash the layer of ore from the surface of the drum into the trough D<sup>8</sup>. The resultant mixture of ore and fresh solvent solution is then led from the trough D<sup>8</sup> into a second receptacle E which may if desired be similar to the receptacle C, but which should preferably be arranged to retain the material for a longer time than does the receptacle C. This receptacle E may also be provided with means for agitating the mixture. From the receptacle E the mixture of ore and the second solvent solution passes to a second dehydrator F similar in construction to the dehydrator D. From the surface of the drum of this second dehydrator the ore may be washed into the trough F<sup>8</sup> by means of jets of liquid from the pipes F<sup>8</sup> which are connected with a suitable source of supply. This liquid may if desired be a third solvent solution, and when such a third solution is used the mixture preferably passes from the trough F<sup>8</sup> to a washer G where it may be diluted by an incoming stream of pure water. If the washer G is provided the mixture preferably passes from it to a third dehydrator H which may be similar to the dehydrators D and F. In this case, however, the ore is preferably washed from the surface of the drum into the trough H<sup>8</sup> by means of pure water instead of by means of a solvent solution. From H<sup>8</sup> the mixture of ore and water with a small residue of solvent solution and of values is discharged as tailings.

In the drawings I have shown a closed system for handling the value containing and barren solutions, but it will be understood that such a system is not essential, so far as my present invention is concerned.

As has been before pointed out, there is connected with each dehydrator a vacuum pump. These vacuum pumps are indicated by D', F' and H', respectively. There is also connected with each dehydrator a precipitation box to which is passed the solvent solution withdrawn from the mixture by the dehydrator and in which the values contained in the solution are extracted. These precipitation boxes are represented by D<sup>6</sup>, F<sup>6</sup> and H<sup>6</sup>, respectively. From the precipitation box H<sup>6</sup> a part of the barren solution is pumped to the cleaning and mixing pipes F<sup>6</sup> of the dehydrator F. The remainder passes on and joins a part of the barren solution from the precipitation box F<sup>6</sup>. This combined barren solution from the boxes H<sup>6</sup> and F<sup>6</sup> is pumped to the cleaning and mixing pipes D<sup>6</sup> of the dehydrator D. The remainder of the barren solution from the precipitation box F<sup>6</sup> passes on and is joined by the barren solution from the precipitation box D<sup>6</sup>. This combined barren solution

from the boxes F<sup>6</sup> and D<sup>6</sup> is pumped into 65 the receptacle B. From the receptacle B the solutions are returned to the tube mill A and the receptacle C. A sufficient quantity of water is supplied to the washer G to offset such losses of liquid as occur at the dehydrator H. Fresh solvent is added at B in sufficient quantities to maintain the proper strength of solvent solution throughout the apparatus and also to offset the loss which occurs in the tailings. 75

What I claim is:

1. The herein described process of ore treatment which consists in mingling an ore mass with a solvent solution to permit the solvent to dissolve a portion of the values from the ore, separating the solution from the ore by a process, as a result of which the ore is left on a surface, removing the ore from the said surface by means of a stream of fresh solvent solution, permitting the said fresh solvent solution to act on the ore which it removes to dissolve further values therefrom, separating the said second solution from the ore, and extracting the values from the said first and second solutions, substantially as set forth. 80

2. The herein described process of ore treatment which consists in mingling an ore mass with a solvent solution to permit the solvent to dissolve a portion of the values 85 from the ore, separating the solution from the ore, subjecting the ore mass, after the said solution has been separated from it, to the action of a jet of fresh solvent solution, whereby the ore mass is broken up and intimately mixed with the said second solution, permitting the said fresh solvent solution to act on the ore to dissolve further values therefrom, separating the said second solution from the ore and extracting the values 90 from the said first and second solutions, substantially as set forth. 100

3. The herein described process of ore treatment which consists in part in the mingling of an ore mass with a solvent 110 liquid to permit the solvent to dissolve a portion of the values from the ore, the separation of the said liquid from the ore, and the subsequent subjection of the ore to the action of a second liquid, the said separation 115 of the first liquid from the ore resulting in the collection of the ore on the surface, and the said subjection of the ore to the action of a second liquid being initially effected by forcing a stream of the said second liquid 120 against the ore on the said surface to remove it therefrom, substantially as set forth.

4. The herein described process of ore treatment which consists in mingling a body of ore with a solvent liquid to permit the 125 solvent to dissolve a portion of the values from the ore, separating the greater portion of the solvent liquid from the ore by a

process as the result of which the ore and the smaller portion of the solution are left in a mass on a surface, removing the said mass from the said surface by means of a stream 5 of fresh liquid whereby the part of the first liquid remaining in the mass is diluted, separating the liquid from the said resulting mixture, and extracting the values from

both of the said separated liquids, substantially as set forth.

In testimony whereof I affix my signature, <sup>10</sup>  
in presence of two witnesses.

CYRUS ROBINSON.

Witnesses:

H. J. G. MASTER,  
DAVID SCOTT.